

## UNITED STATES PATENT OFFICE

2,316,083

## LUBRICANT

Clarence M. Loane, Hammond, Ind., James W. Gaynor, Chicago, Ill., and Lawson W. Mixon, Hammond, Ind., assignors to Standard Oil Company, Chicago, Ill., a corporation of Indiana

No Drawing. Application March 24, 1941,  
Serial No. 384,942

8 Claims. (Cl. 252—48)

The present invention relates to improvements in additives for mineral oils and in particular to an improved phosphorus containing additive for mineral oils and to the method of preparing the same.

In copending applications, Serial No. 384,940, filed March 24, 1941, and Serial No. 384,941, filed March 24, 1941, there are respectively described as additives to mineral oils phosphorus sulfide-hydrocarbon reaction products and neutralized phosphorus sulfide-hydrocarbon reaction products which are effective in inhibiting the deterioration of mineral oils and the attendant formation of sludge, carbon and varnish-like deposits and the method of preparing the additive.

While the phosphorus sulfide-hydrocarbon reaction products as described in the aforesaid copending applications are very effective in inhibiting the deterioration of mineral oils and in preventing the formation of sludge, carbon and/or varnish-like deposits in internal combustion engines during use, they possess a characteristic odor which may be considered objectionable by users of oils containing such additives.

It is an object of the present invention to provide a method of improving the odor of phosphorus sulfide-hydrocarbon reaction products without decreasing the effectiveness of the reaction products. It is a further object of the invention to provide a substantially odorless phosphorus sulfide-hydrocarbon reaction product which is effective in inhibiting the deterioration of mineral oils and which is effective in preventing the formation of sludge, carbon and/or varnish-like deposits in internal combustion engines during use.

We have discovered that the foregoing objects can be attained by reacting the phosphorus sulfide-hydrocarbon reaction product or the neutralized reaction product with an agent having an active hydrogen atom at elevated temperatures, for example, from about 200° F. to about 600° F., and preferably from about 300° F. to about 400° F., either undiluted or in solution in oil or other suitable solvents. Illustrative of the type of agents having an active hydrogen atom at elevated temperatures which are well suited for the herein-described purpose are steam, alcohols, ammonia and amines.

The phosphorus sulfide used in the preparation of the additive can be any phosphorus sulfide, such as, for example,  $P_2S_3$ ,  $P_2S_5$ ,  $P_4S_7$ ,  $P_4S_3$ , etc. and preferably,  $P_2S_5$ .

The hydrocarbon reactants can be paraffins, olefins, or olefin polymers, aromatics, or alkyl

aromatics, cyclic aliphatics, petroleum fractions such as lubricating oil fractions, petrolatums, waxes, cracked cycle stocks, condensation products of petroleum fractions, solvent extracts of petroleum fractions, etc.

The paraffin hydrocarbons can be those obtained from petroleum oils such as bright stock residuums, lubricating oil distillates, petrolatums, or paraffin waxes. We may also halogenate any of the foregoing paraffins and condense the same with aromatic hydrocarbons in the presence of anhydrous inorganic halides, such as aluminum chloride, zinc chloride, boron fluoride and the like.

15 As examples of high molecular weight olefinic hydrocarbons which we may employ as reactants are cetene, ( $C_{16}$ ), cerotene ( $C_{26}$ ), melene ( $C_{30}$ ), and mixed high molecular weight alkenes obtained by cracking petroleum oils.

20 As starting materials for the production of olefin polymers, we can employ the individual olefins themselves, mixtures of olefins, or mixtures of olefins and non-olefinic compounds. For example, the olefinic starting material can be butylenes, amylanes, refinery gases containing normally gaseous olefins and cracked distillates or other relatively low-boiling hydrocarbon mixtures containing normally liquid olefins and mixtures of normally liquid olefins containing 25 substantial amounts of dissolved normally gaseous olefins. We may also employ olefins obtained by the cracking of paraffin wax or by the dehalogenation of alkyl halides, particularly long chain alkyl halides.

30 The polymers referred to above may be those obtained by polymerizing olefinic hydrocarbons in the presence of catalysts such as sulfuric acid, phosphoric acid, aluminum chloride, zinc chloride, boron fluoride and other catalysts of the Friedel-Crafts type. For example, we can employ the polymers resulting from the treatment of mono-olefins, preferably iso-mono-olefins such as isobutylene and isoamylene, and/or the copolymers obtained by the polymerization of hydrocarbon mixtures containing low molecular weight iso-olefins and normal olefins, preferably those of less than six carbon atoms.

35 We can also employ as the starting material the polymer or synthetic lubricating oil obtained by polymerizing unsaturated hydrocarbons resulting from the vapor phase cracking of paraffin waxes in the presence of aluminum chloride. This is fully described in United States Patents 1,995,260, 1,970,002 and 2,091,398. Still another 40 type of olefin polymer which can be employed is

the polymer resulting from the treatment of vapor phase cracked gasoline and/or gasoline fractions with sulfuric acid or solid absorbents such as fuller's earth whereby unsaturated polymerized hydrocarbons are removed. We may also employ as a starting material the polymers resulting from the volatilization of hydrocarbons as described, for example, in United States Patents 2,197,768 and 2,191,787.

Another class of compounds which may be used as starting materials is the aromatic hydrocarbons such as for example benzene, naphthalene, toluene, xylene, diphenyl and the like, or alkylated aromatic hydrocarbons such as, for example, an alkyl substituted benzene in which the alkyl radical has at least four carbon atoms and preferably at least eight carbon atoms such as a long chain paraffin wax.

The phosphorus sulfide-hydrocarbon reaction product may be obtained by reacting a phosphorus sulfide, for example,  $\text{P}_2\text{S}_5$ , with any of the above described hydrocarbons at temperatures of from about 200° F. to about 500° F. and preferably from about 300° F. to about 400° F. and preferably in a non-oxidizing atmosphere, such as an atmosphere of nitrogen. From about 1.0% to about 50% and preferably from about 5% to about 25% of the phosphorus sulfide may be used. If an excess of the phosphorus sulfide is used the reaction product may be freed of the excess phosphorus sulfide by filtering or by diluting with a solvent such as hexane, filtering and subsequently removing the diluent.

The phosphorus sulfide-hydrocarbon reaction product as above obtained, normally shows a titratable acidity which is neutralized when the reaction product is treated with a basic reagent. The phosphorus sulfide-hydrocarbon reaction product when neutralized with a basic reagent having a metal constituent is characterized by the presence or retention of the metal constituent of the reagent. Other metal constituents, such as heavy metal constituents, may be introduced into the neutralization product by reacting the same with a salt of the desired heavy metal.

The term "neutralized phosphorus sulfide-hydrocarbon reaction product" as used herein means a phosphorus sulfide-hydrocarbon reaction product having at least about 1% of its titratable acidity reduced by the reaction with a basic reagent and includes the neutralized phosphorus sulfide-hydrocarbon reaction products containing a metal constituent resulting from said neutralization or resulting from the reaction of a heavy metal salt with the phosphorus sulfide-hydrocarbon reaction product treated with a basic reagent.

The phosphorus sulfide-hydrocarbon reaction product may be neutralized by treating the reaction product with a suitable basic compound such as a hydroxide, a carbonate, or an oxide of an alkaline earth metal or an alkali metal, preferably calcium oxide, potassium hydroxide, or sodium hydroxide. Other basic reagents may be used such as, for example, ammonia or an alkyl or aryl substituted ammonia, such as amines. The neutralization may be carried out in a non-oxidizing atmosphere. As aforesaid when the phosphorus sulfide-hydrocarbon reaction product is neutralized with a basic compound having a metal constituent the neutralized reaction product is characterized by the presence of the metal constituent of the basic reagent. Neutralized reaction products containing a heavy

metal constituent such as, for example, tin, titanium, aluminum, chromium, cobalt, iron and the like, may be obtained by reacting a salt of the desired heavy metal with the phosphorus sulfide-hydrocarbon reaction products which have been treated with a basic reagent. When the neutralization is accomplished with a polyvalent basic metal, such as lime, a product having excess basicity may be obtained.

Both the phosphorus sulfide-hydrocarbon reaction product and the neutralized reaction product, particularly if the latter is incompletely neutralized, possess a characteristic odor which they impart to the lubricant to which they are added. While this does not in any way impair the effectiveness of the compounds in inhibiting the formation of sludge and varnish, it may be objectionable from a sales viewpoint. These products can be substantially freed of this odor by reacting the same with a compound having an active hydrogen atom at an elevated temperature, for example, from about 100° F. to 600° F. and preferably from about 300° F. to 400° F. until a substantial portion of the sulfur is removed as hydrogen sulfide, and the product is substantially odorless. While we may employ compounds such as alcohols, ammonia, and/or amines we prefer to employ steam. Thus, the aforesaid reaction products can be readily freed of the odor by blowing steam through the reaction products either in an undiluted state or in solution in oil or other suitable solvent while maintaining the mixture at the aforesaid temperatures.

Treating the phosphorus sulfide-hydrocarbon reaction products with a compound having an active hydrogen atom, such as steam, at an elevated temperature, results in the final product containing substantially smaller amounts of sulfur. This, however, has substantially no effect on the sludge and varnish inhibiting properties of the product.

The method of preparing the phosphorus sulfide-hydrocarbon reaction product and the method of subsequently deodorizing the same will be illustrated by the following specific examples, which are given merely by way of illustration and not intended to limit the scope of the present invention.

#### EXAMPLE I

50 A mineral lubricating oil derived from a so-called Winkler crude oil, and having a gravity of 25.6 A. P. I., a Saybolt Universal viscosity at 100° F. of 285 to 300 seconds, a flash of not less than 400° F. and a pour point of -5° F. was mixed with 9% of phosphorus pentasulfide and the mixture heated at a temperature of from 100° F. to 400° F. for about three hours and maintained at the maximum temperature for an additional hour. The reaction product was then diluted with 50% of an SAE 20 motor oil and blown with steam at a temperature of 340-350° F. for about three hours. The final product was substantially free of any odor.

#### EXAMPLE II

65 A portion of the phosphorus pentasulfide-lubricating oil reaction product of Example I before being steam blown was diluted with 50% of an SAE 20 motor oil and was treated with 3% of potassium hydroxide at a temperature of 180° F. for two hours. At the end of the two hour heating period the temperature was raised to 340° F.-380° F. and maintained within this temperature range for three more hours, and the product was blown with steam within this same

temperature range for three more hours. The final product containing phosphorus and potassium, was substantially odor-free.

### EXAMPLE III

A cracked cycle stock, recovered as bottoms from a bubble tower, and having a Saybolt Universal viscosity at 100° F. of 53 seconds, a gravity of 23.2 A. P. I., an initial boiling point of 408° F., and a 90% distillation point of 734° F., was mixed with 9% of phosphorus pentasulfide and the mixture heated at a temperature of from about 300-400° F. The mixture was then dissolved in hexane, filtered, and the filtrate distilled to remove the hexane. The product was then diluted with 50% of an SAE 20 motor oil and blown with steam at a temperature of 340-380° F. until substantially no hydrocarbon sulfide was evolved. This product was substantially odor-free.

### EXAMPLE IV

An isobutylene polymer having a Saybolt Universal viscosity at 210° F. of about 3000 seconds was heated with 10% of phosphorus pentasulfide at a temperature of about 380° F. for eight hours. The reaction product so obtained was cooled, 3% of KOH was added, and the mixture was heated at 180° F. for two hours. At the end of the two hour period the temperature was raised to about 340-350° F. and maintained within this temperature range for three hours. This product had a characteristic odor and showed the following analysis:

|            | Percent | 35 | 30 |
|------------|---------|----|----|
| Phosphorus | 3.04    |    |    |
| Sulfur     | 3.97    |    |    |
| Potassium  | 2.1     |    |    |

The above product was diluted with an equal volume of an SAE 20 motor oil and steam blown for three and one-half hours at temperatures of from about 340-350° F. At the end of this period the product was substantially free of any characteristic odor, and showed approximately the same phosphorus and potassium content but showed substantially no sulfur.

### EXAMPLE V

The olefin polymer used in Example IV was treated with 10% phosphorus pentasulfide at a temperature of 380° F. for eight hours. The phosphorus pentasulfide-olefin polymer reaction product was then diluted with an equal volume of an SAE 20 motor oil and treated with 3% of potassium hydroxide at a temperature of 180° F. for two hours. At the end of the two hours heating period the temperature was raised to 340-380° F. and the product was steam blown within this temperature range for three hours. The final product was substantially free of sulfur and the characteristic odor, and contained substantially the same amount of phosphorus and potassium as the product in Example IV.

### EXAMPLE VI

The P<sub>2</sub>S<sub>5</sub>-olefin polymer reaction product was obtained in the manner described in Example IV. The reaction product was diluted with an equal volume of an SAE 20 motor oil and treated with 6% of KOH at a temperature of 180° F. for two hours. The temperature was then raised to about 340-350° F. and maintained within this range for three additional hours, and the product was then blown with steam while within this temperature range for three more hours. A prod-

uct substantially free of the characteristic odor was obtained.

The effectiveness of the deodorized phosphorus sulfide-hydrocarbon reaction products in improving the stability of lubricating oils may be demonstrated by a test described as follows: Two hundred and fifty cc. of the oil to be tested is heated at 330° F. to 332° F. in a 500 cc. glass beaker in the presence of five square inches of copper and ten square inches of iron. Four glass rods of six millimeter diameter are suspended in the oil which is stirred at about 1300 R. P. M. with a glass stirrer having a 40° blade pitch. At stated intervals oil samples are taken and the sludge, acidity and viscosity values determined. The glass rods are also inspected for evidence of varnish formation thereon. Varnish values are based on a visual rating in which glass rods free of any varnish are given a rating of 10, heavily coated rods are given a rating of 1, and rods having coatings between these extremes are given intermediate values between 1 and 10.

The following oils were subjected to the above test:

- 25 Oil A—Control (high grade SAE 20 motor oil).  
 Oil B—Oil A+1% of the deodorized product of Example IV.  
 Oil C—Oil A+1% of the deodorized product of Example V.

TABLE I

| Oil   | Vis. <sup>1</sup> increase | Sludge mg./10 g. oil |         |         |         | Acidity mg. KOH/g. oil |         |         |         | Varnish <sup>2</sup> |         |  |
|-------|----------------------------|----------------------|---------|---------|---------|------------------------|---------|---------|---------|----------------------|---------|--|
|       |                            | 48 hrs.              | 24 hrs. | 48 hrs. | 72 hrs. | 24 hrs.                | 48 hrs. | 72 hrs. | 24 hrs. | 48 hrs.              | 72 hrs. |  |
|       |                            |                      |         |         |         |                        |         |         |         |                      |         |  |
| Oil A | 607                        | 30                   | 762     | ---     | 3.7     | 9.0                    | ---     | 8       | 2-3     |                      |         |  |
| Oil B | 71                         | 0                    | 0       | 77      | 1.4     | 2.5                    | 3.4     | 10      | 10      | 10                   |         |  |
| Oil C | 131                        | 0                    | 0       | 72      | 1.7     | 1.8                    | 3.4     | 10      | 10      | 10                   |         |  |

<sup>1</sup> Saybolt Universal viscosity at 100° F.

<sup>2</sup> 10=no deposit; 1=very heavy deposit.

The above data show the marked improvement obtained by the addition of small amounts of the deodorized phosphorus sulfide-hydrocarbon reaction product to a high grade SAE 20 motor oil.

The effectiveness of the deodorized phosphorus sulfide-hydrocarbon reaction products in inhibiting the formation of carbon, sludge and/or varnish in internal combustion engines is demonstrated by the following data obtained in an engine test conducted in a standard six cylinder spark-ignition engine operating for sixty hours at 35 B. H. P. and 3000 R. P. M. and an oil sump temperature of about 285° F. At the end of each test period the engine was dismantled and given a visual engine rating in which a rating of 10 means that the engine parts had substantially the same appearance at the end of the test as at the start of the test, while an engine rating of 1 means that the engine parts are very badly coated. An engine rating of intermediate value between 1 and 10 means that the appearance of the engine parts after the test is between these extremes. In the tabulation below the visual ratings are given on the following oils.

- 70 Oil A—Control (high grade SAE 20 motor oil).  
 Oil B—Oil A+1/4% deodorized reaction product of Example VI.  
 Oil C—Oil A+3/4% deodorized reaction product of Example VI.  
 Oil D—Oil A+1% deodorized reaction product of Example V.

TABLE II  
ACCELERATED ENGINE TEST  
Visual engine ratings at end of 60 hours

| Oil samples             | A   | B   | C   | D  |
|-------------------------|-----|-----|-----|----|
| Piston varnish.....     | 5   | 6   | 10  | 10 |
| Sludge deposits.....    | 6   | 8   | 9   | 10 |
| Ring belt carbon.....   | 5   | 9   | 10  | 10 |
| Under crown carbon..... | 5   | 6   | 10  | 10 |
| Overall rating.....     | 5.3 | 7.2 | 9.8 | 10 |

The above data demonstrate the marked improvement in engine cleanliness obtained with motor oils containing small amounts of deodorized phosphorus sulfide-hydrocarbon reaction products.

The deodorized reaction products are also effective in inhibiting corrosion of metals, particularly of hard metal alloys, such as alloys of the cadmium-silver type used in bearings.

While we may use the deodorized phosphorus sulfide hydrocarbon reaction products in lubricating oils, which may be used in such oils in amounts of from about 0.001% to 10.0% and preferably from about 0.01% to about 3.0%, our invention is not limited to such use, since these products may be used in other petroleum products, such as insulating oils, white oils, greases, waxes, etc. to inhibit the oxidation, sludging and deterioration thereof.

Although we have described preferred embodiments of our invention, other modifications may be made without departing from the scope and spirit of the invention, and we do not wish to limit our invention to the specific examples set forth herein, except insofar as the same is defined by the following claims.

We claim:

1. A lubricant comprising a mineral lubricating oil and a small amount of the product obtained by reacting a phosphorus sulfide with a hydrocarbon, neutralizing the reaction product resulting therefrom with a basic reagent whereby a neutralized phosphorus and sulfur-containing reaction product is obtained, and subsequently blowing the neutralized phosphorus sulfide-hydrocarbon reaction product with steam at a temperature of from about 200° F. to about 600° F. to obtain a substantially sulfur-free product.

2. A lubricant as described in claim 1 in which the hydrocarbon is a petroleum oil fraction.

3. The method of inhibiting the formation of sludge, carbon and varnish in an internal combustion engine lubricated with a mineral lubricating oil comprising lubricating the internal combustion engine with a lubricant comprising a mineral lubricating oil normally susceptible to form sludge, carbon and varnish during use in an internal combustion engine, and a small amount of the product obtained by reacting a phosphorus sulfide with a hydrocarbon, neutralizing the resulting reaction product with a basic reagent whereby a neutralized phosphorus and sulfur-containing product is obtained and subsequently treating the neutralized reaction product with a compound having an active hydrogen atom at an

elevated temperature above about 100° F. to obtain a final product having a substantially lower sulfur content than the initial neutralized reaction product.

4. The method of inhibiting the formation of sludge, carbon and varnish in an internal combustion engine lubricated with a mineral lubricating oil, comprising lubricating the internal combustion engine with a lubricant comprising a mineral lubricating oil normally susceptible to form sludge, carbon and varnish during use in an internal combustion engine, and a small amount of the product obtained by reacting a phosphorus sulfide with a hydrocarbon, neutralizing the resulting reaction product with a basic reagent whereby a neutralized product containing phosphorus and sulfur is obtained and subsequently blowing the neutralized reaction product with steam at an elevated temperature above about 200° F. to obtain a substantially sulfur-free product.

5. A lubricant comprising a hydrocarbon lubricating oil and a small amount of the product obtained by reacting a phosphorus sulfide with a hydrocarbon, neutralizing with a basic reagent whereby a neutralized product containing phosphorus and sulfur is obtained, and subsequently treating said reaction product at a temperature above about 100° F. with a compound having an active hydrogen atom to obtain a product having a substantially lower sulfur content than the initial reaction product.

6. A new composition comprising a hydrocarbon oil and the product obtained by the process comprising reacting a phosphorus sulfide with a hydrocarbon, whereby a product containing phosphorus and sulfur is obtained, neutralizing with a basic reagent and treating the reaction product at a temperature above about 100° F. with a compound having an active hydrogen atom to obtain a final product having a substantially lower sulfur content than the initial reaction product.

7. A new composition comprising a hydrocarbon oil and the product obtained by reacting a phosphorus sulfide with a hydrocarbon, neutralizing the reaction product resulting therefrom with a basic reagent having a metal constituent whereby a phosphorus and sulfur-containing product having a metal constituent is obtained and subsequently blowing the neutralized reaction product with steam at a temperature above about 200° F. to obtain a substantially sulfur-free product.

8. A new composition comprising a hydrocarbon oil and the product obtained by the process comprising reacting a phosphorus sulfide with a hydrocarbon whereby a phosphorus and sulfur-containing product is obtained, neutralizing with a basic reagent having a metal constituent, and treating the reaction product at a temperature above about 100° F. with a compound having an active hydrogen atom to obtain a substantially sulfur-free product.

CLARENCE M. LOANE.  
JAMES W. GAYNOR.  
LAWSON W. MIXON.